

1

2,977,208

## GAS-PRODUCING COMPOSITION

Aubrey Edward Harper, Glasgow, James Grigor, Coatbridge, and Edward Graham Cooke, West Kilbride, Scotland, assignors to Imperial Chemical Industries Limited, London, England, a corporation of Great Britain

No Drawing. Filed Mar. 12, 1957, Ser. No. 645,643

Claims priority, application Great Britain Apr. 21, 1956

8 Claims. (Cl. 52—5)

This invention relates to improvements in or relating to gas-producing compositions and more particularly to ammonium nitrate compositions capable of self-sustained non-detonating gas-producing reaction.

When compositions capable of self-sustained non-detonating gas-producing reaction are burned in a vented vessel the rate of reaction normally increases with the pressure in the vessel in accordance with a burning rate law as expressed by an exponential equation of the form  $R = bP^n$  where  $R$  is the linear rate of burning,  $P$  is the pressure and  $b$  and  $n$  are constants for the system. The value of the pressure-independent factor  $b$  varies with the initial temperature of the charge, and relations such as

$$b = \frac{b'}{1 - CT}$$

may be used to express this variation. When all factors affecting the rate of burning of a charge are kept constant with the exception of the initial temperature of the charge the equilibrium pressure generated in the vented vessel when said burning rate law is obeyed may be expressed by

$$p = \left[ \frac{K}{1 - CT} \right]^{1/n}$$

where  $K$  is a constant depending on the shape and nature of the charge and the size of the venting orifice. For compositions with the same temperature coefficient  $C$ , it follows from the above equation that for a given temperature range the difference between the equilibrium pressures operative at two temperature levels of a charge is greatest for high values of  $n$ , and least for low values of  $n$ . It is desirable for many purposes, e.g. for charges for use in rocket motors that the operating pressure should be substantially constant over a considerable temperature range and much effort has been expended without success so far to find agents for compositions based on ammonium nitrate which effectively lower the pressure exponent " $n$ ".

It has now been found that compounds of iron, nickel and cobalt are effective agents for lowering the value of " $n$ " of ammonium nitrate charges capable of self-sustained non-detonating gas-producing reaction.

According to the present invention ammonium nitrate charges capable of self-sustained non-detonating gas-producing reaction are characterized in that they include a minor proportion of at least one compound of a metal from the transition elements of the eighth group of the Periodic Classification of the elements, namely iron, cobalt and nickel.

Said ammonium nitrate charges are capable of self-sustained non-detonating gas-producing reaction preferably due to the inclusion therein of a compound of chromium as for instance chromium sesquioxide, a chromate or dichromate, particularly ammonium dichromate.

Compounds of iron, cobalt and nickel suitable in the compositions of the invention include ferrous oxalate, ferrous carbonate, ferrous sulphide, iron oxides, ferrous lactate, ferrous citrate, ferrous hydrogen citrate, ferrous

5

formate, ferrous tartrate, ferric oxalate, potassium ferric oxalate, nickel oxalate, nickel carbonate, nickel formate, cobalt hydroxide, cobalt chromate and cobalt oxalate. It is, however, preferred to include salts of organic acids on account of their superior properties. Of the three metals iron is preferred mainly on account of the superior activity of its salts and ferrous oxalate is particularly useful.

It would seem that it is usually desirable that the compositions of the invention should employ a potassium salt, that the effect of each agent depends on the oxygen value of the composition, and that if any particular ammonium nitrate gas producing composition has to be used it is usually necessary to determine by experiment which agent is the most suitable. Furthermore the charges of the invention need not contain a fuel if the agent is, for instance, ferrous oxalate.

The amount of said compound included is normally of the order of 1 to 10% by weight of the composition. 20 The optimum amount is dependent on the compound and on the nature and make-up of the remainder of the composition and also on the pressure range of interest. The charges of the invention can be given a low exponent " $n$ " particularly for the range of pressures between 300 lb./sq. in. and 1000 lb./sq. in. which range is particularly useful for rocket motor applications.

The invention is illustrated by the following examples in which all parts are by weight.

30

### Example 1

Pressed charges are made of the following compositions, namely 6 parts of a hydrocarbon wax, 92 parts of a 9:1 mixture of ammonium nitrate and potassium nitrate, 2 parts of ammonium dichromate and  $x$  parts of ferrous oxalate.

35

These charges are then made to undergo a self-sustained gas-producing reaction under different constant operating pressures in a vented vessel and the rate of burning at these different pressures measured. The logarithm of each operating pressure is plotted against the logarithm of the corresponding burning rate and the slope of each straight portion of the graph produced gives the value of the pressure exponent " $n$ " for each straight portion.

40

45 The effect of increasing concentration of ferrous oxalate in such charges is shown in the following table which relates concentration of ferrous oxalate and corresponding values of " $n$ " at an arbitrary operating pressure of 400 lb./sq. in. (abs.).

|    | Parts ferrous oxalate ( $x$ ) per 100+ $x$ parts of composition | Pressure exponent " $n$ " at 400 lb./sq. in. (abs.) |
|----|-----------------------------------------------------------------|-----------------------------------------------------|
| 55 | 0.0                                                             | 0.66                                                |
|    | 1.0                                                             | 0.51                                                |
|    | 2.0                                                             | 0.43                                                |
|    | 3.0                                                             | 0.40                                                |
|    | 4.0                                                             | 0.29                                                |
|    | 4.3                                                             | 0.15                                                |
|    | 4.6                                                             | 0.00                                                |
|    | 5.0                                                             | 0.00                                                |
|    | 6.5                                                             | 0.00                                                |
| 60 | 9.0                                                             | 0.71                                                |

### Example 2

Pressed charges are made of the following compositions, namely 6 parts of a hydrocarbon wax, 92 parts 65 9:1 ammonium nitrate/potassium nitrate mixture, 2 parts potassium dichromate and  $x$  parts ferrous oxalate. These charges are then made to undergo a self-sustained thermal decomposition as in Example 1 to obtain graphs of the kind obtained in Example 1. The effect of increasing concentration of ferrous oxalate in such charges on the pressure exponent " $n$ " for an arbitrary operating

pressure of 400 lb./sq. in. (abs.) is shown in the following table.

| Parts ferrous oxalate (x) per 100+x parts of composition | Pressure exponent "n" at 400 lb./sq. in. (abs.) |
|----------------------------------------------------------|-------------------------------------------------|
| 0                                                        | 0.63                                            |
| 2                                                        | 0.49                                            |
| 3                                                        | 0.52                                            |
| 4                                                        | 0.38                                            |
| 4.6                                                      | 0.00                                            |

### Example 3

The effect on the pressure exponent "n" for an arbitrary operating pressure of 400 lb./sq. in. (abs.) of ferrous oxalate at its optimum concentration in various ammonium nitrate compositions is shown in the following table.

| Fuel                          | Fuel, parts by weight | Ammonium nitrate/potassium nitrate (9:1) parts by weight | Ammonium dichromate, parts by weight | Ferrous oxalate, parts by weight | Pressure exponent "n" at 400 lb./sq. in. (abs.) |                        |
|-------------------------------|-----------------------|----------------------------------------------------------|--------------------------------------|----------------------------------|-------------------------------------------------|------------------------|
|                               |                       |                                                          |                                      |                                  | Ferrous oxalate present                         | Ferrous oxalate absent |
| Anthraquinone                 | 12.4                  | 85.6                                                     | 2.0                                  | 5.0                              | 0.00                                            | 0.68                   |
| p-Nitroaniline                | 18.14                 | 78.86                                                    | 3.0                                  | 5.0                              | 0.00                                            | 0.54                   |
| An aniline-formaldehyde resin | 5.85                  | 91.15                                                    | 3.0                                  | 5.0                              | 0.00                                            | 0.50                   |
| Terephthalic acid             | 18.7                  | 78.3                                                     | 3.0                                  | 4.0                              | 0.00                                            | 1.00                   |
| Trinitrostilbene              | 20.0                  | 77.0                                                     | 3.0                                  | 5.0                              | 0.00                                            | 0.57                   |
| None                          | 0                     | 92.0                                                     | 2.0                                  | 2.0                              | 0.00                                            | 0.30                   |

### Example 4

The effect on the pressure exponent "n" for an arbitrary operating pressure of 400 lb./sq. in. (abs.) of various agents at their optimum concentration in an ammonium nitrate composition which includes 6 parts hydrocarbon wax as a fuel, 2 parts ammonium dichromate as catalyst and 92 parts of a 9:1 ammonium nitrate/potassium nitrate mixture and which in the absence of an agent has a pressure exponent "n" at an arbitrary operating pressure of 400 lb./sq. in. (abs.) of 0.66 is shown in the following table.

| Additive                 | Parts by weight | Pressure exponent "n" at 400 lb./sq. in. (abs.) |
|--------------------------|-----------------|-------------------------------------------------|
| Ferrous tartrate         | 5.0             | 0.00                                            |
| Ferrous formate          | 4.0             | 0.00                                            |
| Ferrous citrate          | 5.0             | 0.00                                            |
| Ferrous hydrogen citrate | 5.0             | 0.00                                            |
| Ferrous glycolate        | 5.0             | 0.31                                            |
| Ferrous malate           | 5.0             | 0.33                                            |
| Nickel carbonate         | 5.0             | 0.29                                            |
| Nickel oxalate           | 6.3             | 0.42                                            |
| Cobalt hydroxide         | 4.0             | 0.10                                            |
| Cobalt chromate          | 2.0             | 0.45                                            |

### Example 5

A pressed charge is made having a composition 6 parts of a hydrocarbon wax, 91 parts 9:1 ammonium nitrate/potassium nitrate mixture, 3 parts chromium sesquioxide and 4 parts ferric oxalate. The pressure exponent "n" for this composition is 0.00 at an arbitrary operating pressure of 400 lb./sq. in. abs. while a similar composition from which the ferric oxalate is omitted has a pressure exponent "n" of 0.50 at the same pressure.

### Example 6

A pressed charge is made having a composition 5.5 parts of a hydrocarbon wax, 92.5 parts ammonium nitrate, 2 parts ammonium dichromate and 4.0 parts potassium ferric oxalate. The pressure exponent "n" of this composition is 0.00 at an arbitrary operating pressure of 400 lb./sq. in. abs. whereas the pressure exponent "n" of a similar composition from which the potassium

4 ferric oxalate is omitted has a pressure exponent 0.51 at the same pressure.

### Example 7

The effect of variation of initial temperatures of an ammonium nitrate charge of composition 6 parts of a hydrocarbon wax, 92 parts 9:1 ammonium nitrate/potassium nitrate mixture, and 2 parts ammonium dichromate with and without 5 parts ferrous oxalate on the operating pressure is carried out as follows. Charges of 1.5 inch diameter are fired in a vented vessel so that the initial temperature of the charges lies in the range from -28° C. to 62° C. and the burning rates determined for a series of operating pressures. For the charges at each temperature the logarithm of the rate of burning is plotted against the logarithm of the operating pressure. A collection of linear graphs with the same pressure exponent "n" can thus be obtained for said

range of charge temperatures. From these curves the rates of burning for each charge temperature at a particular arbitrary pressure can be obtained. A curve is now constructed connecting the reciprocal of these rates of burning with the absolute temperature of the charge. The reciprocal of the intercept of the curve so obtained on the absolute temperature axis is numerically equal to the temperature coefficient C. From this value for C the percentage change in operating pressure/° C. rise ( $\pi_k$ ) for any charge of said composition can be calculated by making use of the following equation

$$\pi_k = \frac{100C}{(1-CT)(1-n)}$$

The values of  $\pi_k$  thus obtained for said compositions with and without ferrous oxalate can now be used to calculate the change in operating pressure which will result from changing the charge temperature from -28° C. to 62° C. This is illustrated in the following table wherein the initial operating pressures are arbitrarily chosen as 400 lb./sq. in. absolute.

| Agent present   | C       | $\pi_k$ | Operating pressure, lb./sq. in. (abs.); Initial temperature of charge -28° C. | Calculated operating pressure, lb./sq. in. (abs.); Initial temperature of charge +62° C. |
|-----------------|---------|---------|-------------------------------------------------------------------------------|------------------------------------------------------------------------------------------|
| None            | 0.00183 | 1.11    | 400                                                                           | 796                                                                                      |
| Ferrous oxalate | 0.00180 | 0.38    | 400                                                                           | 537                                                                                      |

It is seen from said table that the change in operating pressure between the temperature limits of -28° C. and 62° C. is considerably less for the composition which includes ferrous oxalate in comparison with the composition which does not include ferrous oxalate.

What we claim is:

1. In a conventional gas-producing composition capable of self-sustained, non-detonating, gas-producing reaction and consisting essentially of ammonium nitrate, the improvement comprising the addition to said composition of from about 1% to 10% by weight of a salt selected from the group consisting of ferrous oxalate,

ferrous malate, ferrous glycolate, ferrous carbonate, ferrous sulphide, ferrous lactate, ferrous citrate, ferrous hydrogen citrate, ferrous formate, ferrous tartrate, ferric oxalate, potassium ferric oxalate, nickel oxalate, nickel carbonate, nickel formate, cobalt hydroxide, cobalt chromate and cobalt oxalate, and a potassium salt selected from the group consisting of potassium nitrate and potassium dichromate.

2. A gas-producing composition as claimed in claim 1, which includes a fuel selected from the group consisting of hydrocarbon wax, anthraquinone, p-nitroaniline, anilineformaldehyde resin, terephthalic acid, and trinitrostilbene.

3. A gas-producing composition as claimed in claim 2 which includes a compound of chromium, selected from the group consisting of chromium sesquioxide, chromates and bichromates.

4. A gas-producing composition as claimed in claim 3 wherein the compound of chromium is a bichromate.

15

10

20

5. A gas-producing composition as claimed in claim 4 wherein the bichromate is ammonium bichromate.

6. A gas-producing composition as claimed in claim 3 wherein the compound of chromium is a chromate.

7. A gas-producing composition as claimed in claim 3 wherein the compound of chromium is chromium sesquioxide.

8. In a conventional gas-producing composition capable of self-sustained, non-detonating, gas-producing reaction and consisting essentially of ammonium nitrate, the improvement comprising the addition to said composition of from about 1% to 10% by weight of potassium ferric oxalate.

References Cited in the file of this patent

UNITED STATES PATENTS

|           |               |               |
|-----------|---------------|---------------|
| 2,159,234 | Taylor        | May 23, 1939  |
| 2,637,274 | Taylor et al. | May 5, 1953   |
| 2,712,989 | Maisner       | July 12, 1955 |
| 2,740,702 | Mace          | Apr. 3, 1956  |